# EUROPEAN PATENT SPECIFICATION

(11) **EP 0 714 248 B1**
(45) Date of publication and mention of the grant of the patent: **06.05.1999**
(21) Application number: 94927171.2
(22) Date of filing: 15.08.1994
(51) Int. Cl.: A46B 13/02, B08B 1/04

(54) **NONWOVEN CLEANING BRUSH**
REINIGUNGSBÜRSTE AUS VLIESSTOFF HERGESTELLT
BROSSE DE NETTOYAGE NON TISSEE

(30) Priority: 19.08.1993 AU 44761/93
(43) Date of publication of application: 05.06.1996
(73) Proprietor: MINNESOTA MINING AND MANUFACTURING COMPANY, St. Paul, Minnesota 55133-3427 (US)
(72) Inventor: ALLAN, James, M., Toronto, Ontario M6R 1R4 (CA); BRANDLEY, Barry, A., Warrimoo, NSW 2774 (AU)
(74) Representative: Warcoin, Jacques
(86) International application number: US9409228
(87) International publication number: WO9505101

(56) References cited:
- EP-A- 0 138 556
- EP-A- 0 227 375
- WO-A-94/04738

## Description

### Technical Field

The present invention relates to a nonwoven thermally bonded fiber compressed brush construction suitable for use in caustic mill environments such as in steel strip mills, for example. More specifically, the invention relates to a brush for use in caustic environments wherein the brush is made from a plurality of compressed annular sections made of bicomponent nonwoven fibers. The brushes of the present invention are made of fibers that can withstand extremely caustic environments without requiring resinous coatings, binders or the like.

### Background Art

Prior to electrolytic tin plating, steel strip must be thoroughly cleaned. This is done on a continuous basis in steel strip mills by passing the strip through a hot caustic cleaning tank and then through hot water rinse tanks. Brushes are commonly used in the cleaning process to agitate the surfaces of the steel strip.

Historically, the aforementioned brushes have been made from any of a variety of materials. Until recently, bristled brushes were commonly used in the cleaning process and typically had natural vegetable fiber bristles. For example, brushes having tampico bristles made from a coarse grass-like plant grown in the region around Tampico, Mexico (hereinafter "tampico bristled brushes") had enjoyed widespread use in steel strip cleaning applications. Bristled brushes may also include bristles of a synthetic construction such as polypropylene, for example. Bristled brushes, however, experienced a short service life in the caustic environment of steel strip mills.

About ten years ago, a cleaning brush made of a compressed body formed of a multiplicity of ganged 5 segments of nylon nonwoven web fabric was developed and sold in Australia by the assignee's subsidiary company, 3M Australia. These brushes were found to have an effective service life two to three times that of the tampico bristled brushes. The Australian brush is made from an air laid randomly formed web of 13 to 15 denier nylon staple of length 38 millimeters. The nylon web is needletacked to increase its density and strength, and the web is thoroughly impregnated with a phenolic resin solution as a binder which, when cured, provides the web with some resistance to highly caustic conditions. This type of brush construction has been utilized for about the last ten years.

However, the phenolic bonded nylon web brush has also exhibited some shortcomings in the caustic environments in which it has been used. Although it generally enjoyed a much longer useful life than the tampico bristled brushes, the nylon web brushes are known to degrade and generate waste or "fluff" as a result of the gradual breakdown under hot caustic conditions (typically pH 13 and 80°C) of the protective phenolic resin binder coating the nylon fibers. The fluff is caused by the release of the nylon staple fibers. The generation of fluff is problematic because it is difficult to clean out of the steel mill cleaning lines and it tends to block filters.

It was also proposed in EP 227 375 assigned to 3M a polyolefin fiber roll comprising a cylindrical body formed of a multiplicity of segments of a nonwoven web of randomly laid entangled polyolefin fiber including an adhesive binder which bonds adjacents fibers together with a chemically resistant bond at points of contact. This prior art forms the preamble of independent claim 1.

Because of the noted problems with cleaning brushes, there is a need for an improved cleaning brush for use in the caustic environments of steel strip mills and the like. Moreover, there is a need for a cleaning brush which has an improved resistance to caustic solutions to thereby avoid the aforementioned degradation of the phenolic resin material and the resulting fluff caused by the destruction of the brush fibers in the caustic environment.

### Disclosure of Invention

The present invention overcomes the noted problems in the art by providing a rotary brush suitable for use in cleaning steel strip rolls and the like in caustic environments, the brush comprising:
a cylindrical body rotatable about its longitudinal axis, said body comprising a compressed stack formed of a plurality of like-oriented annular sections, each section assembled about a central carrier, the sections each comprising a nonwoven web of crimped bi-component fibers comprised of a first polymer component and a second polymer component having a melting temperature lower than the melting temperature of said first polymer component, said first polymer component and said second polymer component attached to one another within each section by melt bonding, said body having a density of between about 50 and about 250 kg/m³.

The fibers making up the compressed annular sections are preferably a combination of polyolefins (e.g. polypropylene and polyethylene) but may also include polyesters and other materials. The annular sections are preferably needle tacked prior to melt bonding. Spacers may be interposed between the annular sections so that the finished brush will include a plurality of annular sections and spacers in a predetermined ratio.

A preferred method of manufacturing the rotary brushes of the present invention comprises:
preparing an air laid web of crimped bicomponent fibers comprising a first polymer component and a second polymer component having a melting temperature lower than the melting temperature of said first polymer component; bonding said first and second polymer components to one another within said web by heating said web to a temperature sufficient to soften said second polymer component and cause melt bonding between said polymer components within said web;
preparing a plurality of annular sections from said nonwoven web; orienting said plurality of annular sections for rotation about a common axis; compressing said plurality of sections along said common axis with a force sufficient to achieve a compacted configuration of said sections having a density of between about 50 and about 250 kg/m³; and restraining said annular sections in said compacted configuration.

Those skilled in the art will more fully understand the details of the invention upon consideration of the remainder of the disclosure including the detailed description of the preferred embodiments and the appended claims.

### Brief Description of Drawings

In describing the preferred embodiments of the invention, reference is made to the various figures wherein:
Figure 1(a) is a plan view of one surface of an annular section of a nonwoven web suitable for inclusion in a rotary brush body according to a first embodiment of the present invention;
Figure 1(b) is a plan view of a surface of a spacer suitable for inclusion in a rotary brush body according to a first embodiment of the present invention;
Figure 1(c) is an exploded view of the elements of a rotary brush body according to a first embodiment of the invention;
Figure 1(d) is a perspective view of a completed rotary brush body according to a first embodiment of the invention;
Figure 2(a) is a plan view of an annular section of a nonwoven web suitable for inclusion in a rotary brush body construction according to a second embodiment of the invention;
Figure 2(b) is a plan view of a surface of a spacer suitable for use in a rotary brush body according to a second embodiment of the invention;
Figure 2(c) is an exploded view of the elements of a rotary brush according to a second embodiment of the invention; and
Figure 2(d) is a perspective view of the completed rotary brush according to the second embodiment of the invention.

### Detailed Description

Details of the preferred embodiments of the invention are now to be described in some detail. It will be understood by those skilled in the art that the structural details of these embodiments are not limiting in any way but are merely illustrative of the features of the invention. In describing the preferred embodiments, reference is made to the various figures wherein the structural features of the invention are identified by reference numerals and wherein identical reference numerals indicate identical structures.

Referring to the various figures, figures 1 and 2 illustrate, respectively, first and second embodiments of a compressed cleaning brush made of a nonwoven thermally bonded fiber web. Figures 1(a)-(d) show various features of a first embodiment of the invention, showing the brush 30 and its components in a tie-bolt construction. Figures 2(a)-(d) illustrate another embodiment of the invention showing the same brush material utilized in a bonded brush construction 40. In one aspect of the invention, the web includes no phenolic resin binders. As those skilled in the art will appreciate, it is also conceivable that the brushes described herein could be made into a flap brush type construction as well as the compressed section type. It will also be appreciated that the spacers described herein may not be essential in certain type brushes such as smaller brushes, for example.

In both of the embodiments described herein, a nonwoven web is used to prepare the annular sections 10 and 20. In the web, it is preferred that bicomponent fibers be used without additional resins (e.g. phenolic resins) or the like to either protect or bind the fibers of the web. Preferred web fibers include certain polymer fibers such as polyolefin fibers, polyester fibers and combinations thereof. More preferably, polyolefin bicomponent fibers are used and most preferably polyethylene and polypropylene crimped staple fibers. In order to achieve a satisfactory brush construction which is resistant to physical damage in the caustic environments in which it will be used while achieving a desired cleaning effect, the fiber diameter can be important. Polyolefin fibers in deniers from about 3 to about 40 denier are preferred. The fiber length can range from being virtually continuous to being of finite length. Crimped polyolefin staple fibers having lengths from about 25 millimeters to about 64 millimeters and more preferably from about 38 to about 50 millimeters have been useful in preparing webs using conventional web forming equipment. The fibers may be only slightly crimped and the nature of the fiber crimp includes conjugate or helical crimps. Typically the fibers are thermoplastic bi-component, i.e. sheath and core type or side-by-side type, one component preferably being polypropylene and the other preferably polyethylene. It is also contemplated that polyester bicomponent fibers may be used.

The preferred construction of the web includes no additional resinous materials to bond or protect the fibers of the web. An important aspect of the invention is the manufacture of a bicomponent web wherein the fibers are melt bonded to one another at the fiber contact points within the web. In webs made from the above mentioned preferred combination of polyolefins, for example, the web is typically heated to the temperature of the lower melting point polyethylene component while the higher melting point polypropylene component maintains its dimensions during the heating step. During this heating step, the melted polyethylene fibers bond with the polypropylene at the contact points of the fibers within the web and the web experiences only minimal shrinkage during bonding. Preferred webs for the brush construction are those made in web basis weights from about 100 grams per square meter ("gsm") to about 500 gsm and those having a web thickness of from about 5 millimeters to about 25 millimeters. The above described nonwoven webs may be manufactured in a known manner by using a RANDO WEBBER brand machine (Rando Machine Corporation, Macedon, NY) or a FIBER LOCKER brand machine (James Hunter, North Adams, Mass.).

For additional web strength (i.e. tensile and tear strengths) a needle punching or needle tacking operation performed on the web before melt bonding has been found to be advantageous. Needle tacking is a known technique which uses barbed or felting needles to further entangle the fibers of a nonwoven web by forcing the needles into the web in a predetermined manner. Where needle tacking has been employed, satisfactory webs have been achieved by using a needle tacker machine fitted with a multiplicity of needles, typically 15 x 18 x 30 x 3.5 CB Foster felting needles fitted to the needle board. One preferred needle bar layout includes five rows spaced apart at distances of 8.5 mm, 8.5 mm, 10 mm and 6.5 mm and with the needles in each row evenly spaced at a distance of 12.5 mm.

After punching, the web is transported by conveyors through a preheated oven. A 25 meter long, center fed (e.g. counter current air flow towards the web inlet end and concurrent towards the exit) oven which is gas fired with an air flow at its inlet duct of about 8000 cubic feet/minute (227 cubic meters/minute) and about 4000 cfm at the exit ducts (113 cubic meters/minute) has been used with satisfactory results. Air flow is deflected through the web with angled baffles above and below a carrier mesh belt and the web is heated to the softening or melting temperature of one of the component fibers. Where polypropylene/polyethylene fibers are used, the web is heated to a temperature from about 142°C to about 148°C to induce heat fusion of the fibers. Those in the art will appreciate that the temperature of the oven may be varied over a range of temperatures depending upon the weight of the web and the speed at which the web is fed through the oven. It has been found that satisfactory webs are produced by feeding the nonbonded web material having a weight of about 200 gsm at a line speed of four meters per minute through a 25 meter long oven maintained at a temperature of about 142°C. As the weight of the web and/or the speed at which it is carried though the oven increases, the temperature of the oven must also be increased. A 250gsm web, for example, has been adequately bonded at a temperature of about 148°C when conveyed through the oven at a conveyor speed of five meters per minute.

The bonded web is cooled on exiting the oven with an air knife and passed through a dancing nip roller from which it enters a festoon accumulator prior to being wound onto a master roll or "jumbo". Annular sections 10, 20 are then punched from the manufactured web. The sections 10, 20 are punched from the web in a variety of diameters which will typically vary between about 200 millimeters and about 600 millimeters, depending on brush requirements as well as the available physical space in the cleaning line(s) where the finished brush is to be installed. It will be appreciated that the invention does not require any real limit to the web diameter or to the brush length other than what might be imposed by engineering design considerations.

The web sections 10, 20 are formed with center apertures 70, 80 which may include opposing squared-off keyway slots 90 (Figure 1a) to fit over a key element on a support shaft. Additional slots 92 may be provided to engage long tie-bolts (or axle bolts) 100 which hold the brush components together during the assembly process. Where a glued brush construction is required, tie bolts 100 are not used and the sections 20 and spacers 50 are adhered to a steel core 110 as shown in Figures 2(a)-(d), for example.

Spacers 50, 60 are provided for positioning between web sections. The spacers 50, 60 are typically made from a thermoplastic material such as polypropylene, and are provided with a center hole configuration similar (and usually identical) to the apertures 70, 80 of the webs 10, 20. As shown, the spacers are provided with a smaller outer diameter than the annular sections 10 and 20. The spacers are positioned between annular sections along an assembly shaft such as the axle bolts 100 in a predetermined number of spacers per finished brush and at a predetermined number of annular sections per spacer. The section to spacer ratio in the brushes of Figures 1 and 2, for example, is 3:1 and the loading of annular sections is typically 12.5 sections per 25 millimeters of brush length. Those skilled in the art will appreciate that this brush loading and the section to spacer ratio is not limiting in any way. It is contemplated that preferred brush loadings could range between about 5 and about 20 sections per 25 millimeters and the preferred section to spacer ratios could range from about 1:0 to about 5:1. The use of spacers 50, 60 within the construction of the brushes disclosed herein is generally desired because the spacers allow the annular web sections 10, 20 in the finished brush some freedom to move laterally at their peripheral portions for proper cleaning operations while also firmly reinforcing the annular sections 10, 20 along their inner diameters. Spacers made of polypropylene having an outer diameter of 200 millimeters, an inner diameter of 109 mm and a thickness of 1.9 mm have been satisfactory.

In the embodiment of figure 1c and 1d, the annular sections 10 and the spacers 50 are assembled along the axle bolts 100 between end flanges 120. In the embodiment of figure 2c and 2d, the sections 20 and the spacers 150 are positioned along the core 60. After a predetermined number of spacers and annular sections have been assembled as described above, the spacers and the annular sections are compressed under a sufficient force at room temperature to make a dense nonwoven brush structure of a predetermined length which can then be loaded onto working shafts (not shown) for cleaning operations in steel mills. The compacted densities of the brushes of the present invention are preferably at least about 5 kg/m³ and more preferably between about 50 and about 250 kg/m³ and most preferably about 125 kg/m³. The compaction force may be applied by any suitable means available to those in the art. Once the desired compacted density has been attained, the annular sections and the spacers are then restrained in their compacted configuration by any suitable means such as the end flanges 120 or locking collars adapted to be slidable on and mechanically engagable with the axle bolts 100. Similarly, the sections 20 and the spacers 150 of figure 2 may be held on the core 60 by adhesive bonding. The preferred hardness of the finished brushes as measured by the Shore A2 scale is between about 5 and about 25.

In a preferred construction of the present invention, the web is made from a side-by-side bi-component polyethylene/polypropylene staple fiber supplied by Chisso Corporation (Polypropylene Fiber Division, 6-32 Naanoshima 3, Kita-Ku, Osaka 530, Japan) and termed Chisso Type ES. The preferred staple fiber is 18 denier and length 64 millimeters. The preferred web weight is 250gsm. The web may be needle punched at a punch density of about 8 punches/cm² by needletacking at 760 cycles/min and with a penetration of 21 millimeters into the web at a line speed of four meters per minute. Where lines speeds are increased to five meters per minute, for example, the tacker rate should be increased to about 950 cycles/min. Other line speeds may require further adjustments which are within the skill of those practicing in the field. A preferred brush construction 30, 40 includes about 600 annular sections and about 200 polypropylene spacers 50, 60, each about 1.9 millimeters thick to form a 1.2 meter long x 406 millimeters diameter compressed brush.

It has been found that when the brush of the present invention is run in the same hot caustic application as the conventional nylon/phenolic bonded brush, the brush of the present invention exhibited an extended life about 70% greater than the nylon/phenolic brush. The brush of the invention has also been observed to generate reduced "fluff" or waste during normal use in caustic environments. These results reflect a life extension of about 350% along with a significant reduction in mill maintenance when compared with the tampico bristled brushes discussed above.

The following example is illustrative of the manufacture, construction and the durability of a preferred embodiment of the nonwoven brushes of the invention.

### Example

A 250 g/m², 50 mm thick nonwoven fabric is prepared by processing "CHISSO" polyethylene/polypropylene sheath/core staple fiber (Chisso Corporation, Osaka, Japan or Chisso America, Inc., New York, NY), 18 denier x 38 mm length using an air lay machine available under the trade designation "RANDO WEBBER" from Rando Machine Corporation, Macedon, NY. The resulting fabric is consolidated by needle tacking using a conventional needletacker with a needle board loaded to 10 needles per inch (3.9 per cm) with needles designated 15x18x30x3.5 CB, available from Foster Needle Company, Manitowoc, WI. The needle tacker is adjusted to provide 85 mm needle penetration and 49 penetrations/in² (7.6 penetrations/cm²). The thus consolidated fabric is passed at 5 m/min. through a 25 meter long forced-draft bonding oven heated to 148°C. The resulting fabric is about 10 mm thick, is well bonded and relatively stiff, and has no fluffy appearance.

Annular sections of three different diameters are then cut from the consolidated and bonded fabric. The majority of the sections are cut to provide an outer diameter ("o.d.") of 406 mm and an inner diameter ("i.d.") of 109 mm, the i.d. further provided with 4 equiangularly spaced notches to accept an array of 4 axle bolts, and two symmetrical notches to provide a keyway for mounting on an end use shaft. Lesser numbers of sections are cut having outside diameters of 300 mm and 255 mm, all with an inside diameter of 109 mm and with the same array of notches an in the 406 mm sections. The two smaller o.d. sections are used to provide tapered or stepped ends for the final brush. Polypropylene spacers of 200 mm o.d., 109 mm i.d., and thickness of 1.9 mm are cut from polypropylene sheet, also providing the notches to accommodate the axle bolts and shaft keys. Having provided these various sections and the spacers, the cleaning brush of the present invention is now ready for assembly.

Four axle bolts are secured to an end flange in an equiangular array identical to that of the axle bolt notches provided in the sections and spacers. The end flange is also provided with two opposing keyway notches, likewise matching those provided in the sections and spacers. Four 255 mm o.d. annular sections are placed over the axle bolts so that the axle bolts engage the axle bolt notches. A spacer is then placed similarly over the axles bolts, followed by two 300 mm o.d. sections, followed by a spacer, then followed by two 406 mm o.d. sections and subsequently a spacer. This assembly is continued by alternating three 406 mm o.d. sections followed by a spacer until about 250 sections are loaded on the axle bolts. The assembly of sections and spacers is then compressed under a force of about 850 psi (5.9 MPa) and retained by a clamp assembly. This entire loading procedure is then repeated with three 406 mm o.d. sections followed by a spacer until about 600 sections are loaded. The assembly is completed by loading a spacer, two 300 mm o.d. sections, a spacer, four 255 mm o.d. sections, and finally, another end flange. The entire assembly is then compressed under a force of about 850 psi (5.9 MPa) and the end flange is secured. The resulting cleaning brush is 1.2 meters in length.

The cleaning brush is mounted on a keyed shaft and can then be evaluated as a cleaning brush in a plating operation where it is subjected to a heated (80°C) cleaning solution which is highly caustic, typically having a pH of about 13. The brush will perform the cleaning operation adequately, generating virtually no fluff, and will have a useful life of nearly twice that of a conventional nylon/resin brush.

## Claims

1. A rotary brush comprising:
a cylindrical body rotatable (30,40) about its longitudinal axis, said body comprising a compressed stack formed of a plurality of like oriented annular sections (10,20), each section assembled about a central carrier (60,100), characterized in that the sections each comprise a nonwoven web of crimped bi-component fibers comprised of a first polymer component and a second polymer component having a melting temperature lower than the melting temperature of said first polymer component, said first polymer component and said second polymer component attached to one another within each section by melt bonding to each other, said body having a density of between about 50 and about 250 kg/m³.

2. The rotary brush as defined in claim 1 wherein at least one of said sections are needletacked.

3. The rotary brush as defined in claim 1 wherein said first polymer component is polypropylene and said second polymer component is polyethylene.

4. The rotary brush as defined in claim 1 wherein said fibers are side-by-side crimped bicomponent fibers having a denier within the range of about 3 to about 40.

5. The rotary brush as defined in claim 1 wherein each said section has a basis weight in the range of about 100 to about 500 gsm.

6. The rotary brush as defined in claim 1 further comprising at least one spacer (50,150) interposed between adjacent annular sections.

7. The rotary brush as defined in claim 6 wherein said spacers (50, 150) are interposed between adjacent annular sections (10,20) so that the ratio of said sections to said spacers within said brush is from about 1:0 to about 5:1.

8. The rotary brush as defined in claim 6 wherein the first polymer component and the second polymer component comprise materials selected from the group consisting essentially of polyolefins, polyesters and combinations thereof.

9. The rotary brush as defined in claim 8 wherein said sections (10,20) and said at least one spacers compacted along the length of said common axis (60,100) at a density of about 125 kg/m³.

10. A method for preparing a rotary brush for cleaning operations according to claim one, comprising:
preparing an air laid nonwoven web of crimped bicomponent fibers comprising a first polymer component and a second polymer component having a melting temperature lower than the melting temperature of said first polymer component;
bonding said first and second polymer components within said web to one another by heating said web to a temperature sufficient to soften said second polymer component and cause melt bonding between said polymer components within said web;
preparing a plurality of annular sections (10,20) from said nonwoven web;
orienting said plurality of annular sections for rotation about a common axis (60,100);
compressing said plurality of sections along said axis with a compaction force sufficient to achieve a compacted configuration of said sections having a density of between about 50 and about 250 kg/m³; and
restraining said annular sections in said compacted configuration.

11. The process defined in claim 10 wherein the preparing of said air laid web is accomplished using fibers selected from the group consisting essentially of polyolefins, polyesters and combinations thereof.

12. The process defined in claim 10 wherein the preparing of said air laid web is accomplished using polypropylene as said first polymer component and polyethylene as said second polymer component.

13. The process defined in claim 12 wherein said bonding step is accomplished by heating said web to a temperature within a range of about 142°C and about 148°C.

14. The process defined in claim 13 wherein said bonding step is accomplished by passing said web at a rate of about 5 meters/minute through a forced draft bonding oven heated to about 148°C.

15. The process defined in claim 10 wherein the preparing of a plurality of annular sections (10,20) is accomplished by punch cutting annular shapes having a variety of sizes from said web, each of said annular sections prepared to include a central aperture (70,80) dimensioned to receive a shaft (100) therein.

16. The process defined in claim 10 wherein said compressing of said plurality of said sections comprises applying a compressive force to said sections of about 850 MPa.

17. The process defined in claim 16 wherein the density of said sections after said compressing thereof is about 125 kg/m³.

18. The process defined in claims 10 said orienting of said sections includes aligning a predetermined number of said annular sections (10,20) along said common axis (60,100) together with a predetermined number of annular spacers, (50,150) said spacers aligned along said common axis between adjacent annular sections such that the annular section to spacer ratio in the rotary brush is from about 1:0 to about 5:1.

19. The process defined in claim 10 further comprising needletacking said web prior to said bonding thereof, said needletacking carried out using a needle board loaded to a density of 3.9 needles per centimeter.

20. The process defined in claim 19 wherein said needletacking is accomplished with needle penetrations into said web of about 7.6 penetrations/cm² and with the needles on said needle board penetrating about 85mm into said web.

## Patentansprüche

1. Drehbürste mit:
einem zylindrischen Körper (30,40), der um seine Längsachse drehbar ist, wobei der Körper einen komprimierten Stapel aus mehreren gleichartig ausgerichteten ringförmigen Teilen (10,20) aufweist, von denen jeder um einen zentralen Träger (60,100) herum angeordnet ist,
dadurch gekennzeichnet, daß die Teile jeweils eine Vliesbahn aus gekräuselten Bikomponenten-Fasern aufweisen, die eine erste Polymer-Komponente und eine zweite Polymer-Komponente enthalten, welche eine Schmelztemperatur unterhalb der Schmelztemperatur der ersten Polymer-Komponente hat, wobei die erste Polymer-Komponente und die zweite Polymer-Komponente innerhalb jedes Teils durch Schmelzverbondung aneinander befestigt sind und der Körper eine Dichte zwischen ungefähr 50 und ungefähr 250 kg/m³ hat.

2. Drehbürste nach Anspruch 1, bei der mindestens einer der Teile vernadelt ist.

3. Drehbürste nach Anspruch 1, bei der die erste Polymer-Komponente Polypropylen ist und die zweite Polymer-Komponente Polyethylen ist.

4. Drehbürste nach Anspruch 1, bei der die Fasern nebeneinanderliegende gekräuselte Bikomponenten-Fasern mit einer Denier-Stärke im Bereich von ungefähr 3 bis ungefähr 40 sind.

5. Drehbürste nach Anspruch 1, bei der jeder Teil ein Basisgewicht im Bereich von ungefähr 100 bis ungefähr 500 gsm hat.

6. Drehbürste nach Anspruch 1, ferner mit mindestens einem Abstandshalter (50,150), der zwischen benachbarten ringförmigen Teilen angeordnet ist.

7. Drehbürste nach Anspruch 6, bei der die Abstandshalter (50,150) derart zwischen benachbarten ringförmigen Teilen (10,20) angeordnet sind, daß das Verhältnis der Teile zu den Abstandshaltern in der Bürste von ungefähr 1:0 bis ungefähr 5:1 beträgt.

8. Drehbürste nach Anspruch 6, bei der die erste Polymer-Komponente und die zweite Polymer-Komponente Materialien aufweisen, die aus der Gruppe gewählt sind, die im wesentlichen aus Polyolefinen, Polyestern und Kombinationen aus diesen besteht.

9. Drehbürste nach Anspruch 8, bei der die Teile (10,20) und der mindestens eine Abstandshalter entlang der Länge der gemeinsamen Achse (60,100) mit einer Dichte von ungefähr 125 kg/m³ komprimiert sind.

10. Verfahren zum Herstellen einer Drehbürste für Reinigungsoperationen gemäß Anspruch 1, mit den folgenden Schritten:
Herstellen eines Blasvlieses aus gekräuselten Bikomponenten-Fasern, die eine erste Polymer-Komponente und eine zweite Polymer-Komponente aufweisen, welche eine Schmelztemperatur unterhalb der Schmelztemperatur der ersten Polymer-Komponente hat;
Verbonden der ersten und zweiten Polymer-Komponenten in dem Vlies durch Heizen des Vlieses auf eine Temperatur, die ausreichend ist, um die zweite Polymer-Komponente zu erweichen und eine Schmelzverbondung zwischen den Komponenten in der Bahn zu bewirken;
Herstellen mehrerer ringförmiger Teile (10,20) aus der Vliesbahn;
Ausrichten der ringförmigen Teile zur Drehung um eine gemeinsame Achse (60,100);
Komprimieren der Teile entlang der Achse der Teile mit einer Kompaktierungskraft, die ausreicht, um eine kompaktierte Konfiguration der Teile mit einer Dichte zwischen ungefähr 50 und ungefähr 250 kg/m³ zu erzielen; und
Rückhalten der ringförmigen Teile in der kompaktierten Konfiguration.

11. Verfahren nach Anspruch 10, bei dem das Herstellen des Blasvlieses unter Verwendung von Fasern erfolgt, die aus der im wesentlichen aus Polyolefinen, Polyestern und Kombinationen aus diesen bestehenden Gruppe gewählt sind.

12. Verfahren nach Anspruch 10, bei dem das Herstellen des Blasvlieses unter Verwendung von Polypropylen als erste Polymer-Komponente und Polyethylen als zweite Polymer-Komponente durchgeführt wird.

13. Verfahren nach Anspruch 12, bei dem der Verbondungsschritt durch Heizen des Vlieses auf eine Temperatur im Bereich zwischen ungefähr 142°C und ungefähr 148°C durchgeführt wird.

14. Verfahren nach Anspruch 13, bei dem der Verbondungsschritt durchgeführt wird, indem die Bahn mit einer Rate von ungefähr 5 Metern/Minute durch einen auf ungefähr 148°C geheizten Druckluftstrom-Verbondungsofen hindurchgeführt wird.

15. Verfahren nach Anspruch 10, bei dem das Herstellen mehrerer ringförmiger Teile (10,20) durchgeführt wird, indem Ringformen mit verschiedenen Größen aus der Bahn gestanzt werden, wobei jeder der ringförmigen Teile derart behandelt wird, daß er eine zur Aufnahme einer Achse (100) bemessene zentrale Öffnung (70,80) aufweist.

16. Verfahren nach Anspruch 10, bei dem das Komprimieren der Teile das Aufbringen einer Kompressivkraft von ungefähr 850 MPa auf die Teile umfaßt.

17. Verfahren nach Anspruch 16, bei dem die Dichte der Teile nach deren Komprimieren ungefähr 125 kg/m³ beträgt.

18. Verfahren nach Anspruch 10, bei dem beim Ausrichten der Teile eine vorbestimmte Anzahl der ringförmigen Teile (10,20) entlang der gemeinsamen Achse (60,100) zusammen mit einer vorbestimmten Anzahl ringförmiger Abstandshalter (50,150) ausgerichtet wird, wobei die Abstandshalter entlang der gemeinsamen Achse zwischen benachbarten ringförmigen Teilen derart ausgerichtet sind, daß das Verhältnis zwischen Ringteil und Abstandshalter in der Drehbürste von ungefähr 1:0 bis ungefähr 5:1 beträgt.

19. Verfahren nach Anspruch 10, bei dem ferner ein Vernadeln der Bahn vor deren Verbondung vorgesehen ist, wobei das Vernadeln mittels eines Nadelbretts durchgeführt wird, das mit einer Dichte von 3,9 Nadeln pro Zentimeter bestückt ist.

20. Verfahren nach Anspruch 19, bei dem das Vernadeln mit Nadel-Einstichen in das Vlies bei ungefähr 7,6 Einstichen/ cm² und bei einer Einstichtiefe der auf dem Brett befindlichen Nadeln in die Bahn von ungefähr 85 mm durchgeführt wird.

## Revendications

1. Brosse rotative comportant:
un corps cylindrique (30, 40) pouvant tourner autour de son axe longitudinal, ledit corps comprenant une pile comprimée formée d'une pluralité de sections annulaires (10, 20) orientées de la même façon, chaque section assemblée autour d'un support central (60, 100), caractérisée en ce que les sections comportent chacune un tissu non tissé de fibres à deux composants, frisées, constituées d'un premier composant polymère et d'un second composant polymère présentant une température de fusion inférieure à la température de fusion dudit premier composant polymère, ledit premier composant polymère et ledit second composant polymère attachés l'un a l'autre a l'intérieur de chaque section par liaison l'un à l'autre par fusion, ledit corps ayant une densité valant entre environ 50 et environ 250 kg/m³.

2. Brosse rotative comme définie dans la revendication 1, dans laquelle au moins l'une desdites sections a subi un traitement de pénétration par des aiguilles.

3. Brosse rotative comme définie dans la revendication 1, dans laquelle ledit premier composant polymère est du polypropylène et ledit second composant polymère est du polyéthylène.

4. Brosse rotative comme définie dans la revendication 1, dans laquelle lesdites fibres sont des fibres à deux composants côte à côte, frisées, d'un n° tex d'environ 0,33 à environ 4,44 (environ 3 à environ 40 deniers).

5. Brosse rotative comme définie dans la revendication 1, dans laquelle chaque dite section a un poids de base d'environ 100 à environ 500 g/m².

6. Brosse rotative comme définie dans la revendication 1, comportant en outre au moins un écarteur (50, 150) interposé entre des sections annulaires adjacentes.

7. Brosse rotative comme définie dans la revendication 6, dans laquelle lesdits écarteurs (50, 150) sont interposés entre des sections annulaires adjacentes (10, 20) de façon que le rapport entre lesdites sections et lesdits écarteurs de ladite brosse vaille d'environ 1:0 à environ 5:1.

8. Brosse rotative comme définie dans la revendication 6, dans laquelle le premier composant polymère et le second composant polymère comportent des matériaux choisis dans le groupe essentiellement constitué de polyoléfines, de polyesters et de leurs combinaisons.

9. Brosse rotative comme définie dans la revendication 8, dans laquelle lesdites sections (10, 20) et lesdits écarteurs dont il y a au moins un sont compactés selon la longueur dudit axe commun (60, 100) sous une densité d'environ 125 kg/m³.

10. Procédé de préparation d'une brosse rotative pour des opérations de nettoyage conformément à la revendication 1, comportant:
préparer un tissu non tissé, obtenu par jet d'air, de fibres à deux composants, frisées, comprenant un premier composant polymère et un second composant polymère ayant une température de fusion inférieure à la température de fusion dudit premier composant polymère;
lier l'un à l'autre ledit premier et ledit second composants polymères à l'intérieur dudit tissu en chauffant ledit tissu à une température suffisante pour ramollir ledit second composant polymère et provoquer une liaison par fusion entre lesdits composants polymères à l'intérieur dudit tissu;
préparer une pluralité de sections annulaires (10, 20) à partir dudit tissu non tissé;
orienter ladite pluralité de sections annulaires en vue d'une rotation autour d'un axe commun (60, 100);
comprimer ladite pluralité de sections selon ledit axe avec une force de compactage suffisante pour obtenir une configuration compactée desdites sections d'une densité valant entre environ 50 et environ 250 kg/m³;
retenir lesdites sections annulaires dans ladite configuration compactée.

11. Processus défini dans la revendication 10 dans lequel la préparation dudit tissu obtenu par jet d'air se fait en utilisant des fibres choisies dans le groupe essentiellement constitué de polyoléfines, de polyesters et de leurs combinaisons.

12. Processus défini dans la revendication 10, dans lequel la préparation dudit tissu obtenu par jet d'air se fait en utilisant du polypropylène comme dit premier composant polymère et du polyéthylène comme dit second composant polymère.

13. Processus défini dans la revendication 12, dans lequel ladite étape de liaison se fait en chauffant ledit tissu à une température valant entre environ 142°C et environ 148°C.

14. Processus défini dans la revendication 13, dans lequel ladite étape de liaison se fait en faisant passer ledit tissu à la vitesse d'environ 5 mètres/minute à travers un four de liaison à courant d'air forcé, chauffé à environ 148°C.

15. Processus défini dans la revendication 10, dans lequel la préparation d'une pluralité de sections annulaires (10, 20) se fait en découpant au poinçon, dans ledit tissu, des formes annulaires présentant une variété de dimensions, chacune desdites sections annulaires préparée pour inclure une ouverture centrale (70, 80) dimensionnée pour y recevoir un arbre (100).

16. Processus défini dans la revendication 10, dans lequel ladite compression de ladite pluralité desdites sections consiste à appliquer auxdites sections une force compressive d'environ 850 MPa.

17. Processus défini dans la revendication 16, dans lequel la densité desdites sections après leur compression est d'environ 125 kg/m³.

18. Processus défini dans la revendication 10, dans lequel ladite orientation desdites sections inclut l'alignement d'un nombre prédéterminé desdites sections annulaires (10, 20) selon ledit axe commun (60, 100) en même temps que d'un nombre prédéterminé d'écarteurs annulaires (20, 150), lesdits écarteurs alignés selon ledit axe commun entre les sections annulaires adjacentes de façon que le rapport entre lesdites sections annulaires et lesdits écarteurs de ladite brosse rotative soit d'environ 1:0 à environ 5:1.

19. Processus défini dans la revendication 10, comportant en outre pour ledit tissu un traitement de pénétration par des aiguilles avant sadite liaison, ledit traitement de pénétration par des aiguilles effectué en utilisant une planche à aiguilles chargée de 3,9 aiguilles par centimètre.

20. Processus défini dans la revendication 19, dans lequel ledit traitement de pénétration par des aiguilles s'accomplit avec des pénétrations d'aiguilles dans ledit tissu d'environ 7,6 pénétrations/cm²_{,} les aiguilles se trouvant sur ladite planche à aiguilles pénétrant dans le tissu sur environ 85 mm.
